

## UNITED STATES PATENT OFFICE

2,382,699

## SLUSHING OIL COMPOSITIONS

Gordon W. Duncan, Scotch Plains, N. J., assignor  
to Standard Oil Development Company, a cor-  
poration of Delaware

No Drawing. Application January 2, 1941,  
Serial No. 372,831

1 Claim. (Cl. 106—14)

This invention relates to slushing compositions, that is, to non-drying compositions of matter for arresting, preventing and inhibiting the corrosion of metals.

The corrosion of a metal is considered the result of chemical reactions between the environment and the metallic surface due to differences in electromotive forces in and about the surface of the metal. By coating metallic surfaces with an inert, impervious film, the development of these electrochemical relations can be impeded and arrested and thus active corrosion prevented. The use of a slushing composition involves the formation of a relatively thick, viscous liquid or semi-solid layer which is easily removable from the surfaces over which it is spread by wiping with a cloth or flushing with a readily available solvent. More durable coatings may be obtained by employing a more viscous oil base and heating the mixture prior to application to allow better treatment of the surface. In no case, however, is the protective layer of the nature of a difficultly-removable varnish-like layer. The use of slushing compositions is particularly advantageous when metallic surfaces have to be temporarily protected such as engine parts during storage or tubing during shipment.

It has now been found that when small amounts of salts of certain nitrogen base compounds and organic acids are incorporated in slushing compositions the composite is characterized by marked anti-corrosive properties and the capacity in many cases of the composites to displace moisture from the metallic surfaces. The compositions of the invention are therefore improved slushing oil compositions which contain in addition to the usual constituents of the nature of a protective base material which may be a fatty compound, a mineral oil of about lubricating consistency or a more resistant non-drying coating material, small amounts of salts of nitrogen base compounds such as the organic amines and heterocyclic nitrogen bases, and organic acids. These new type addition agents are either dissolved or finely dispersed in anti-rust compositions. A type of anti-rust composition which is appreciably improved by the addition thereto of the compounds of this invention is that disclosed in Patent 2,182,992. These compositions are composed of a petroleum oil of lubricating oil consistency blended with a fatty compound, such as degras, and mahogany soap such as an alkaline metal soap of the oil-soluble sulfonates derived from petroleum by treating oils

with concentrated sulfuric acid. The following formula is a specific example:

|                                                                                                                                    | Per cent |
|------------------------------------------------------------------------------------------------------------------------------------|----------|
| 5 Petroleum oil (750 secs. Saybolt at 100° F.)                                                                                     | 85       |
| 50% oil solution of sodium salts of oil-soluble sulfonic acids formed on treating petroleum stocks with concentrated sulfuric acid | 10       |
| Degras                                                                                                                             | 5        |

10 All of the common amines, that is, the readily available primary, secondary and tertiary amines, in combination with fatty or naphthenic acids have been found to be very effective anti-corrosive agents when incorporated in hydrocarbon and fatty base protective compositions. A preferred class of compounds are the salts of those amines boiling above about 150° F. but which are sufficiently basic to form relatively stable soaps with the respective acids. Where water displacement properties are of importance, it has been found desirable to employ those soaps which have affinity for water or appreciable solubility in water. Amines which upon reaction with an organic acid 15 are hydrophilic are the alkyl amines such as phenyl ethanolamine, diethyl ethanolamine or ethyl diethanolamine, the lower molecular weight aliphatic primary amines such as the amyl and hexyl amines and the lower molecular weight 20 heterocyclic nitrogen bases such as pyridine, quinoline and morpholine. The acids which are suitable for reaction with these amines to prepare hydrophilic soaps are the unsaturated fatty acids of between 10 and 20 carbon atoms which react 25 with the particular amine to form a stable compound. Besides this group of unsaturated fatty acids, the naphthenic acids derived from petroleum especially those from the naphtha, gas oil and lubricating oil ranges, are advantageous in 30 this regard. For the preparation of soaps within the scope of this invention however, that is for incorporation in compositions upon which no particular emphasis is laid as to their water displacing ability, any amine which reacts with an organic acid to form a stable compound may be 35 employed. The saturated fatty acids above 25 carbon atoms are the least desirable acid constituents of the soaps suitable for compositions according to the present invention.

40 The amine salts employed in this invention as additives in the various compositions may be prepared by the reaction of the amine or mixture of amines with an organic acid or mixture of such acids. Natural fats may be used as a source 45 of the fatty acids and when so employed the fats 50

may be saponified by heating with the amine at a high temperature and thus the amine salt is prepared directly. The naphthenate salts may be formed from the naphthenic acids derived from any of the naphthenic acid containing mineral oil crudes or fractions thereof. The acids may be extracted from the petroleum distillates by any of the known processes such as by distilling over caustic soda, extracting the sodium naphthenates by aqueous alcoholic solutions, acidifying the resultant solutions and repurifying as desired. The nature of the amine salt formed is determined largely by the process by which it is prepared

The compositions according to the invention comprise the addition of the compounds of the invention, particularly the amine soaps in amounts between 0.25% and 5.0% and preferably between 1% and 3% by weight to mineral or vegetable oil or wax bases. In the case of vegetable oils, such as castor oil, amine soaps in amounts between 1 and 5%, with or without a diluent such as alcohol, are effective rust preventative compositions. Furthermore, these compositions have substantially no effect upon rubber.

The efficacy of coating compositions is evaluated by certain standard tests of which the humidifier test and displacement of various aqueous solutions are the more important.

#### HUMIDIFIER TEST

##### TEST PROCEDURE

Sand blasted panels of hot rolled steel (automobile body sheet steel) are dipped into slushing compound samples, then maintained vertically in a box for 16 hours under ordinary room conditions. Compounds containing petrolatum are applied at temperatures above their melting point and fluid products are applied at room temperatures. The coated panels are then placed and spaced apart in an upright position in a humidifier chamber having a volume of 16 cu. ft. and air of a given humidity and temperature is injected at a rate of 12 cu. ft./hr. In the test the temperature is maintained at 100° F., the humidity at 100%. The time, in hours, for a panel subjected under these conditions to develop a rusting appearance is observed and recorded as the resistance life of the coating composition.

The following data illustrate the rust preventative effectiveness of various compositions:

##### Humidifier test

[100° F.-100% humidity]

|   | Compound                                                                                                                                           | Hours to initial rusting |
|---|----------------------------------------------------------------------------------------------------------------------------------------------------|--------------------------|
| 1 | (a) Coastal SAE 40 lubricating oil.....<br>(b) Coastal + 2% diethylethanolamine oleate.....<br>(c) Coastal + 2% dicyclohexylamine naphthenate..... | 2<br>300+<br>192         |
| 2 | (a) 70% Coastal SAE 40 lubricating oil + 30% petrolatum.....<br>(b) 70% Coastal SAE 40 lubricating oil + 3% dicyclohexylamine naphthenate.....     | 24<br>250+               |
| 3 | (a) Petrolatum.....<br>(b) Petrolatum + 1% dicyclohexylamine naphthenate.....                                                                      | 24-48<br>200+            |
| 4 | (a) Petrolatum + 1% morpholine naphthenate.....<br>(b) Castor oil.....<br>(b) Castor oil + 5% morpholine oleate.....                               | 200+<br>3<br>120         |

#### WATER DISPLACEMENT TEST

##### TEST PROCEDURE

Sand blasted panels of hot rolled steel are dipped in an aqueous solution and while still wet are immediately immersed in the slushing compounds for a period of one minute. The panels are then suspended vertically for 2 hours

in the laboratory atmosphere, then washed with naphtha, and examined for signs of corrosion. In a series of tests, the effects of many different amine soaps in a mixture of 75% petroleum naphtha and 25% SAE 20 mineral lubricating oil were investigated with the following results:

##### Tap water displacement tests

|    |                                                                                                                                                                                                                                                                                                                                                                                                                                                                                                                                                                                           | Corrosion                                                                            |
|----|-------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|--------------------------------------------------------------------------------------|
| 10 | 1. 75% naphtha + 25% SAE 20 lubricating oil (A).....<br>2. A + 2% morpholine naphthenate.....<br>3. A + 2% morpholine oleate.....<br>4. A + 2% morpholine soap of oxidized wax acids, (partially soluble) <sup>1</sup> .....<br>5. A + 2% diethylethanolamine naphthenate.....<br>6. A + 2% diethylethanolamine oleate.....<br>7. A + 2% diethylethanolamine soap of oxidized wax acids (partially soluble).....<br>8. A + 2% dicyclohexylamine naphthenate.....<br>9. A + 2% dicyclohexylamine soap of oxidized wax acids <sup>1</sup> .....<br>10. A + 2% dicyclohexylamine oleate..... | Severe<br>None<br>None<br>Light<br>None<br>None<br>Light<br>Trace<br>Light<br>Medium |

<sup>1</sup> Oxidized wax acids include both unsaturated and saturated fatty acids.

In another test similarly conducted the ability of these agents to displace corrosive solutions other than tap water is evaluated.

##### Corrosion by aqueous solution displacement test

|    | Tap water   | 0.25% hydrogen chloride | Synthetic perspiration <sup>1</sup> | Sea water   |
|----|-------------|-------------------------|-------------------------------------|-------------|
| 35 | Severe..... | Severe.....             | Severe.....                         | Severe..... |
| 40 | None.....   | do.....                 | do.....                             | None.....   |
| 45 | do.....     | Medium.....             | Medium.....                         | Trace.....  |
| 50 | do.....     | Light.....              | None.....                           | None.....   |
|    | do.....     | None.....               | do.....                             | Do.....     |
|    | do.....     | do.....                 | do.....                             | Do.....     |
|    | do.....     | do.....                 | do.....                             | Do.....     |

<sup>1</sup> 0.7% sodium chloride, 0.4% lactic acid, 0.1% urea in distilled water.

The addition agents of this invention are effective as corrosion inhibitors and agents for displacing moisture from metallic surfaces when incorporated in protective base compositions. The resultant compositions are effective for protecting finely polished surfaces and for heavy machinery parts exposed to weathering. Individual compositions have characteristics adapted for the particular uses for which they are to be employed. The consistency of the various compositions is determined by the service requirements and the manner in which the compositions are to be applied to the surfaces to be protected. Thus, in the case of the protection of highly finished metal articles such as cutlery, and the finely ground engine surfaces the compositions may contain in addition to the protective base a volatile material such as gasoline which some time after application of the composition to the surfaces evaporates and leaves behind a layer of protective material of the base and addition agent of this invention. In other cases it is preferable to employ as anti-rust compositions materials of consistencies which are semi-solid or even solid in order to withstand the effects of exposure to heavy rains and other at-

mospheric conditions. In all cases, however, the compositions are readily removed by a wiping or brushing treatment of the surfaces.

Particular uses of compositions of the present invention are for the protection of engine surfaces. Usually automobile engines and parts are assembled and tested before leaving the factory and the surfaces coated with a slushing composition in order to protect them until required for service. By means of the use of the present slushing compositions of suitable consistency and protective quality no deterioration of the engine surfaces and therefore of engine efficiency occurs as the result of storage or delays in shipment through varied atmospheric and climatic conditions. Furthermore, compositions of this invention that are suitable for use in the protection of engine assemblies have suitable solubilities in light lubricating oils which are generally employed as solvents to flush the system before placing the engine in service. An added property of such compositions is that the constituents which are incorporated have no harmful effect upon lubricating oils which are subsequently employed in the lubrication of the engine. The addition agents of this invention as a group do not exert any deleterious effect upon mineral lubricating oils and therefore their incorporation in slushing composi-

tions for engine assemblies is particularly advantageous.

Although the mechanism and operation of the amine soaps in the various compositions are not understood and it is not desired to be limited to any particular theory as to the operation thereof, it is believed that the amine soaps present in the compositions have some effect in neutralizing nascent acids formed near the surface of the metals.

10 It is believed that the soaps have an action different from that when dissolved in water and have capacity to inhibit the development of electrochemical relations in the surface of the metal.

15 It is not intended that this invention be limited to any of the particular examples which have been given for purposes of illustration nor by any of the theories as to the operation of the invention, but only by the appended claims in which it is desired to claim all the novelty inherent in the

20 invention.

What is claimed is:

25 A slushing composition comprising a viscous petroleum fraction to which is added 5% degras, 10% of a 50% oil solution of sodium salts of oil-soluble sulfonic acids formed on treating petroleum stocks with concentrated sulfuric acid and 0.25% to 5% of dicyclohexylamine naphthenate.

GORDON W. DUNCAN.